

# United States Patent [19]

Manfroy et al.

[11]

4,162,044

[45]

Jul. 24, 1979

[54] PROCESS FOR GRINDING COAL OR ORES  
IN A LIQUID MEDIUM

3,934,825 1/1976 Delfosse ..... 241/16  
3,950,182 4/1976 Steel et al. ..... 241/15  
3,989,195 11/1976 Steward ..... 241/16

[75] Inventors: Willy Manfroy, Carmel, Ind.;  
Richard R. Kliment, Midland, Mich.

## FOREIGN PATENT DOCUMENTS

47200 4/1974 Australia ..... 241/16

[73] Assignee: The Dow Chemical Company,  
Midland, Mich.

## OTHER PUBLICATIONS

[21] Appl. No. 932,872

"Chem. Enhancement of Ore Grinding Efficiency,"  
Hartley et al., Battelle, Pacific NW Laboratories, Aug.  
1976, Vail, Colo.

[22] Filed: Aug. 11, 1978

"Crushing and Grinding," G. C. Lowrison, pp.  
106-110, 1974, CRC Press Inc., Cleveland, Ohio.

[63] Continuation-in-part of Ser. No. 853,734, Nov. 21,  
1977, abandoned, which is a continuation-in-part of  
Ser. No. 687,782, May 19, 1976, abandoned.

[51] Int. Cl.<sup>2</sup> ..... B02C 23/18  
[52] U.S. Cl. ..... 241/16; 51/298  
[58] Field of Search ..... 241/15, 16, 18, 20,  
241/30; 51/298

"Computers and Operations Research in Mineral Indus-  
tries" R. Kliment et al., Oct. 1976, 14th International  
Symposium.

[56] References Cited

Primary Examiner—Donald J. Arnold  
Attorney, Agent, or Firm—G. D. Street

## U.S. PATENT DOCUMENTS

|           |         |              |        |
|-----------|---------|--------------|--------|
| 2,905,565 | 9/1959  | Dietz et al. | 241/16 |
| 3,104,068 | 9/1963  | Castelli     | 241/16 |
| 3,252,662 | 5/1966  | Lyons et al. | 241/16 |
| 3,534,911 | 10/1970 | Gwilliam     | 241/16 |
| 3,604,634 | 9/1971  | Windle       | 241/16 |
| 3,648,937 | 3/1972  | Ehrreich     | 241/15 |
| 3,756,979 | 9/1973  | Ventres      | 241/16 |

## ABSTRACT

A process for grinding coal or ores containing metal  
values comprising carrying out said grinding in a liquid  
medium and with a grinding aid comprising an anionic  
polyelectrolyte derived from polyacrylic acid and dis-  
persible in the liquid medium, said grinding aid being  
present in an amount effective to provide increased  
grinding efficiency.

25 Claims, No Drawings

**PROCESS FOR GRINDING COAL OR ORES IN A LIQUID MEDIUM**

**CROSS-REFERERNCE TO RELATED APPLICATIONS**

This application is a continuation-in-part of our pending application Ser. No. 853,734, filed Nov. 21, 1977, now abandoned, which in turn is a continuation-in-part of our application Ser. No. 687,782, filed May 19, 1976, now abandoned.

**BACKGROUND OF THE INVENTION**

The present invention relates to the use of polyacrylic acid-derived polymers as grinding aids to increase the rate of coal or ore-particle breakage in the wet-grinding of solids in mills such as ball, bead, rod or pebble mills, or in autogenous grinding operations.

In the processing of mineral ores and many other solids, the essential step is the comminution of the solids down to the size at which valuable mineral grains are released from the gangue matrix. With the inevitable trend towards working of lower-grade ore deposits, the amounts of minerals liberated tend to decrease and the grinding cost per ton of product increases. This factor alone constitutes a considerable fraction of the overall cost of winning metals and the increase in cost of energy has made grinding costs a very significant factor.

The amount of breakage per unit of time (breakage kinetics) and mass transfer of grinding mineral ores are usually controlled by the addition and removal of water, an excellent medium because of its high polarity, to the mill. When the mass transport of the slurry through the mill decreases, the mill operator takes corrective action by either decreasing the solids feed rate and/or temporarily increasing the amount of water entering the mill. While both actions will prevent the mill from overloading, mill efficiency is reduced because fewer solids are ground per unit of time under such conditions.

Additionally, it is well known that the traditional tumbling mill apparatus used for wet-grinding ores are extremely inefficient in energy utilization, wasting (based on theoretical bond breakage energies) perhaps as much as 90% or more of the energy supplied to the mill. Therefore, even small increases of a few percent in the reduction of size distribution of ore particles and an increase in throughput of ore ground per unit of time would significantly improve the efficiency of grinding and cost of mill operations, especially with respect to energy utilization.

While various methods and chemical agents that act as grinding aids have been employed in efforts to increase grinding efficiencies and economics, these efforts have at best been only partially beneficial and many have even proved to be contradictory in related downstream processing operations. Various chemical agents, e.g., dispersants, surfactants, polysiloxane, organosilicones, glycols, amines, graphite, non-polar liquids and the like have all been utilized and may increase the rate of grinding by preventing particle agglomeration. However, as reported in Perry's Chemical Engineering Handbook, 5th Ed. 1973, at Sec. 8-12, there really is no scientific method of choosing the most effective surfactant. Rather, surfactant lists and kits that can be used for systematic trials are made available.

Chemical agents, such as polyacrylic acid salts, copolymers of acrylic acid and acrylamide, hydrolyzed polyacrylonitrile and the like are known to be useful as

dispersants at low molecular weight ranges. Polymers having a molecular weight from a few thousand up to about 50,000, for example, have been utilized as dispersants in the grinding of calcium carbonate to separate impurities therefrom. See U.S. Pat. No. 3,534,911 and 3,604,634.

**SUMMARY OF THE INVENTION**

The present invention provides a process for grinding coal or ores containing metal values which comprises carrying out the grinding operation in the presence of a liquid medium and a grinding aid comprising polyacrylic or polymethacrylic acid or an anionic derivative thereof, said grinding aid being dispersible in said medium and being employed in an amount effective to provide increased grinding efficiency. The use of such grinding aids results in a substantial increase in the rate of particle breakage and permits higher density (solids) slurries of coal or ore to be ground, thereby achieving a greater volume throughput of solid ground per unit of time with a corresponding increase in the recovery rates of the desired metal value where ores are ground. The resulting improved efficiency in the overall grinding operations, i.e., in the use of mill capacity and particularly in the consumption of energy per unit of product, is achieved with the present grinding aids without encountering a decrease in grinding kinetics normally observed when higher density slurries are ground.

It has also been found that the polyelectrolyte grinding aids of the present invention usually do not detrimentally effect downstream processing operations which are performed, particularly on mineral ores, after the mineral leaves the grinding mill. Thus, for example, the polyelectrolyte grinding aids generally do not detrimentally effect processes such as, for example, froth flotation processes in which select metal values such as copper, lead, zinc or gold are recovered from the ore with the aid of flocculating and deflocculating agents. Neither do the polyelectrolyte grinding aids of the present invention have any counterproductive effects in subsequent operations such as, for example, in pelletizing iron ore. Since the polyelectrolyte is adsorbed on the solids, the system does not contribute to downstream pollution problems upon discharge of the aqueous medium such as might be the case with phosphatic materials, for example.

**DETAILED DESCRIPTION OF THE INVENTION**

The method of the present invention is preferably carried out in the presence of a polar liquid medium in which the grinding aid is sufficiently dispersible to produce an improvement in grinding efficiency, although the use of a liquid medium comprising a liquid which itself is not a solvent for the grinding aid may be feasible provided that a solvent or dispersant for the grinding aid is also present. Accordingly, the term dispersible means the aids are soluble or dispersible in the medium employed to an extent sufficient to provide adsorption thereof on the solid particles and increased grinding efficiency. Water is ordinarily employed and is the preferred medium. The concentration of the solids, e.g., ore or coal, in the liquid medium may vary within wide limits and it is usual to operate with a slurry solids content in the range of from about 40 to about 95, preferably about 50 to about 90, more preferably from 65 to about 88% and most preferably from 70 to about 88,

percent by weight of the slurry. Metal ores which may advantageously be treated according to the present invention include iron, copper, gold, silver, lead, zinc, nickel and the like which can be subjected to a wet-grinding treatment. In a preferred embodiment, an ore containing a metal value is ground according to the process of the invention. In another embodiment, coal is preferably ground according to the invention process.

The polyelectrolyte grinding aid used in the present invention is suitably any polyelectrolyte derived from acrylic acid which is inherently dispersible in the liquid medium employed. Preferably, the polyelectrolyte is dispersible in the liquid medium without the aid of surfactants. Exemplary polyelectrolytes include the water soluble or dispersible polymers or copolymers of acrylic or methacrylic acid or the salts thereof. Preferably, the homopolymers are employed. The salt of the acid may be that of an alkali metal, for example, sodium, potassium, lithium or the like, or may be an ammonium salt. The alkali metal salts, especially the sodium salts, are preferred. Preferably, the grinding aids are employed in the form of water-soluble salts. Preferred grinding aids are the sodium salts of polyacrylic acid of polymethacrylic acid.

Copolymers of acrylic or methacrylic acid with other ethylenically unsaturated monomers such as, for example, acrylamide, vinylacetate, acrylonitrile, methacrylate, ethylacrylate, 2-methylpropanoic acid and the like are also within the scope of the invention. Such copolymers usually contain about 25 weight percent or more of the acrylic or methacrylic acid monomer. Further, those skilled in the art will recognize that some ethylenically unsaturated polymers, such as, for example, acrylamide, are sometimes characterized by a greater or lesser degree of hydrolysis, i.e., contain some free carboxyl groups. This condition is dependent upon the method of manufacture of the polymer, the presence or absence of other minor ingredients in the starting monomer, e.g., acrylic acid, conditions of storage and the like. The polymer products appear to be equivalent whether the carboxyls result from copolymerization of acrylamide with acrylic acid or from hydrolysis of amide groups subsequent to polymerization or copolymerization and grinding aid products resulting from either method are within the scope of the invention. Other additives, such as triethanolamine, for example, can also be added with the acrylic or methacrylic acid polymer as long as the resulting product contains about 50 weight percent or more of the acrylic or methacrylic acid moiety.

Generally, the anionic group of the grinding aid has a pKa of about 8 or less, wherein pKa is a negative logarithm of the acidity constant for the acidic (anionic) group. The average molecular weight (as determined by the Mark Houwink equation) of the water-soluble or dispersible polymers and salts thereof usually ranges from about two or three thousand up to about fifty thousand. Preferably, grinding aids having an average molecular weight of from about 5000 to about 20,000 and more preferably from about 5000 to about 10,000 are employed. The upper limit on molecular weight is not critical, while it is known that some very high molecular weight polymers are difficult to get into solution but that colloidal dispersions thereof can be formed in the medium. Polyelectrolytes which are otherwise insoluble or non-dispersible in the medium are not included within the scope of the invention.

It has been found that the effectiveness of the polyelectrolyte grinding aid relates to the number of anionic groups in the polyelectrolyte. In one means of determination, the number is found to be sufficient if the polyelectrolyte effects a minimum 10% reduction in the low shear viscosity of a slurry when the polyelectrolyte is added to the slurry in an amount sufficient to provide a concentration of 0.06 weight percent of polyelectrolyte based on total mineral solids. By low shear viscosity is meant Brookfield viscosity determined with a Brookfield viscometer using a #D bar at 25° C. and 5 rpm. By slurry it is meant that coal or a mineral is ground to a particle size of 325 mesh and that the concentration of solids in the liquid medium is between about 50 to about 95% by weight. Preferred polyelectrolytes effect at least about a 20% viscosity reduction under such conditions, with the most preferred effecting a viscosity reduction of at least about 40%. So long as viscosity reductions in this range are effected, the number of anionic groups in the polyelectrolyte is not particularly critical. However, as a general rule, the polyelectrolytes advantageously employed have a proportion of anionic groups in the polyelectrolyte such that there are at least about 1, preferably about 2 or more, milliequivalents of anionic moiety per gram of the polyelectrolyte.

Water-soluble polymers of the type exemplified above are known and can be prepared by a variety of methods. Examples of suitable water-soluble polymers include, for example, available products such as, for example, DISPEX N-40® (manufactured by Allied Colloide Manufacturing Company Ltd.), DAXAD® (available from W. R. Grace Co.), TAMOL 850® (Rohm and Haas Co.) and GOODRITE K732® (Goodrich Tire and Rubber Co.) and the like.

Acrylic or methacrylic homopolymers which are especially suitable for use in this invention are readily prepared from the monomer by the action of heat, light, and/or catalysts. Catalysts which are particularly effective for this polymerization include peroxides. The properties and nature of the polymer can be varied over a considerable range by the proper choice of catalysts and/or reaction conditions.

Grinding aids which are preferred in the present invention are most advantageously made by polymerizing the monomer, for example, acrylic acid, in aqueous solution at about 50°-170° C. in the presence of a redox polymerization catalyst system by dispersing acrylic acid and a peroxy catalyst separately and continuously into the aqueous medium at rates such that an effective and substantially constant concentration of the catalyst system is maintained in contact with the acrylic acid throughout the polymerization. A reducing agent can be combined with the acrylic acid and the two added as a single aqueous solution, but preferably, the reducing agent is added separately and continuously as a third stream.

The peroxy catalyst component can be any peroxide useful as a polymerization catalyst. Suitable peroxides, which preferably are water soluble, include hydrogen peroxide, tert-butyl hydroperoxide and salts of per acids such as sodium persulfate, potassium percarbonate, ammonium peracetate, sodium perbenzoate, sodium perborate, and the like.

The concentration of peroxygen-containing catalyst can vary widely within limits of about 0.1-10% based on the entire polymerization mixture and referring to active catalyst present in the system at any one time during the process. Preferably, the amount of aqueous

medium and the rates of addition of catalyst and acrylic acid are adjusted so that a relatively high peroxy catalyst concentration is maintained. Total peroxy catalyst used based on the acrylic acid is preferably about 0.5-5 mole percent. The reducing agent is employed in at least a molar equivalent amount based on the peroxy component and preferably is used in a quantity of about 20-100 percent excess. Both components of the redox catalyst system are preferably added as aqueous solutions of relatively high concentration.

The aqueous polymerization medium is preferably water but it may include up to about 30% by volume of a water-miscible organic solvent such as acetone, a lower alkanol, or dimethyl sulfoxide. Efficient stirring of the polymerization mixture or agitation by other effective means is required so that the streams of peroxy catalyst, reducing agent, and acrylic acid are quickly and thoroughly dispersed and intimately mixed in the polymerization medium. Superatmospheric pressure may be advantageous.

Other modes of polymerization may also be employed. These are well known in the art and the particular process employed is not critical to this invention.

The amount of grinding aid employed to increase grinding efficiency, e.g., the rate and type of ore-particle breakage, e.g., ore classification, which can respectively be described as the "selection" and "distribution" functions of grinding, will vary depending upon certain factors including properties which are unique to coal and each ore. For example, the "selection function", which describes the probability that a particle of any particular size will be broken in a given unit of time, will be affected by any factors which change the probability of particle breakage. Factors such as slurry volume, number and size of grinding media (e.g., balls, rods, etc.), raw ore particle size, mill rpm and the like, as well as ore properties, all affect the probability of successful particle breakage. The properties unique to coal or each ore also affect the "distribution function", that is, the number and size distribution of fragments into which a particle will subdivide when it is broken. Measurement of the number and size distribution of fragments after grinding will allow the calculation of the effect of the aid on the selection and distribution functions which will indicate the effectiveness of the grinding aid added. Further reference to the use of selection and distribution functions in determining the effect of grinding aid materials in wet grinding process can be found in

Klimpel, R. R., and Manfroy, W., "Computer Analysis of Viscosity Effects on Selection for Breakage and Breakage Distribution Parameters in the Wet Grinding of Ores", *14th Int. Sym. on Appl. of Computers in the Mineral Ind.*, Pennsylvania State U., University Park, Pa., October 1976;

Klimpel, R. R., and Manfroy, W., "Grinding Aids for Increased Throughput", *Symposium of Canadian Min. Proc.*, Ottawa, Canada, January 1977;

Klimpel, R. R., and Manfroy, W., "Development of chemical Grinding Aids and Their Effect on Selections-for-Breakage and Breakage Distribution Parameters in the Wet-Grinding of Ores", *Proc. 12th Int. Min. Proc. Congress*, August-September 1977, Sao Paulo, Brazil.

Grinding efficiency can, for example, be determined from the amount of particulate solid of particle size less than 325 mesh (44 micrometers) U.S. Standard, that can be formed from a given liquid slurry of constant volume of liquid and ore solids using the same energy input.

Normally, as the weight percent of ore solids in this slurry is increased, the grinding efficiency of the grinding medium is reduced. Thus, it is critical in the practice of this invention that the amount of polyelectrolyte grinding aid employed be sufficient to reverse the trend towards a lower grinding efficiency as weight percent concentration of ore solids in the slurry is increased.

The liquid slurry preferably contains grinding media wherein the media are as employed in large ore grinding mills such as ball, bead, rod or pebble mills. The media are generally of a size large enough where they do not contribute to an increase in the inherent viscosity of the slurry. Thus, the type of mills under consideration here are distinct from those mills in which paint pigments are ground to an extreme fineness with an extremely small granular grinding medium.

Generally, the effective amount of grinding aid employed to increase the rate of ore grinding can be as low as about 0.002 percent by weight (of actual polymer)

20 based on the dry weight of the ore present. The maximum amount of grinding aid employed is usually limited by economic constraints, i.e., the high cost of the grinding aid. Preferably, the grinding aids of the present invention are employed in the range of from about 0.003 to about 0.08% by weight of actual polymer (i.e., from about 0.03 to about 0.8 milligram per gram) preferably, from about 0.01 to about 0.04% by weight. The optimum amount of aid from an economic and/or utility viewpoint will, of course, depend upon, *inter alia*, the particular ore to be ground and other various factors as described hereinabove. Those skilled in the art can readily ascertain the same according to the procedures set forth herein or others known in the art.

35 In batch operations, grinding periods of from 5 to 10 minutes or longer are usually sufficient to measure an increase in the fineness of grind when using a grinding aid as taught herein. In open cycle continuous grinding operations, the increased throughput and/or increased fineness of grind at constant throughput is readily ascertained. In continuous closed cycle grinding operations, however, much of the ore being ground is continuously recycled through the grinder until the desired degree of fineness is obtained and the actual grinding time per unit of ore can only be calculated on an average residence basis. This will vary with the type of ore used and the amount of grinding required to meet size distribution requirements. With iron ore, for instance, grinding must be continued until the particle size is less than 325 mesh (U.S. Standard), sometimes less than 500 mesh. Again, those skilled in the art of grinding will be able to ascertain the grinding time needed.

Increases in grinding kinetics are determined by measuring the change in the weight and size distribution of fragments obtained per unit of time. An increase in the amount of grinding or fineness of grind as determined by measurement of the particle sizes resulting per unit grinding time means that more grinding takes place. Illustrating the increased grinding rates achieved in another manner, it is readily apparent that if a grinding viscosity of, for example, 50,00 cps is desired and the untreated ore slurry is at 68% solids, one can grind a higher solids density slurry of, for example, 72% solids, by use of a grinding aid without any change in grinding conditions. Increases in the grinding rate of only a percent or two, while numerically small, are highly desirable as they represent truly significant savings in energy costs. According to the methods of the present invention, experimental data indicates that increases of from

about 1 to about 20 percent of the grinding rate can be achieved with the use of grinding aids taught herein.

In determining the usefulness of a particular agent as a grinding aid, various chemicals can be first screened to determine the ability of a particular chemical agent to decrease the viscosity of a finely ground ore. Those agents generally found to decrease the viscosity of the finely ground ore (ground to a particle size of 325 mesh and having a solids concentration between about 50 to 95% by weight) by about 20-25 percent or more are usually subsequently found to be very effective as grinding aids. Generally, the greater the decrease in slurry viscosity, the greater the increase in grinding. However, viscosity data alone is not sufficient by itself to predict that any increase in grinding efficiency will necessarily result or to indicate the degree of any increase in grinding efficiency which might be obtained. This will have to be determined by actual grinding trials. In carrying out actual grinding tests, an ore sample is first ground in a typical ball mill using plain water as a liquid phase. After each grinding run of a predetermined time, the size distribution of the product is determined by wet screening. Enough runs are made with different grinding periods and slurry concentrations so that the change in the weight and size of fragments can be determined. The runs are then repeated incorporating a grinding aid into the slurry and making the same determinations. The changes in the size and weight of fragments as compared with the controls indicate the effectiveness of the grinding aid.

The following examples are presented to illustrate the invention, but are not to be construed as limiting it in any manner whatsoever. The ore slurry percent is based on the weight of solids present in the slurry being treated and the milligrams per gram is based upon the number of milligrams of actual grinding aid per gram of ore.

#### EXAMPLE 1

Various chemical agents were screened to determine the effectiveness thereof in decreasing the viscosity of a finely-ground ore. In such operations, ground ore was mixed with sufficient water to form a viscous slurry, usually between about 100,000 and 150,000 cps. The viscosity of the slurries was measured with the use of a Brookfield viscometer fitted with a crossbar and helipath stand, the helipath slowly moving the revolving crossbar (at 5 rpm) vertically so that the bar continuously encounters undisturbed slurry. A base viscosity curve of untreated slurry is first determined. Then a dilute solution of the test agent is added in 5 small equal increments of 1 cc each to the slurry. The viscosity change is plotted as a function of treatment level and the results compared with the untreated slurries.

In such operations, the viscosity of slurries treated with various levels (mg/gm of ore) of sodium poly-

acrylate and copolymers of polyacrylate and acrylamide were found to be decreased as compared with control samples:

TABLE I

| Ore                        | Aid                    | mg/gm | % Decrease<br>Slurry Viscosity |
|----------------------------|------------------------|-------|--------------------------------|
| 1. Taconite <sup>(a)</sup> | Na polyacrylate        | 0.2   | 40                             |
| 2. Taconite <sup>(b)</sup> | "                      | "     | 31                             |
| 3. Copper <sup>(c)</sup>   | "                      | "     | 42-68 <sup>(d)</sup>           |
| 4. Gold                    | "                      | "     | 75                             |
| 5. Iron <sup>(e)</sup>     | "                      | "     | 57                             |
| 6. Copper <sup>(f)</sup>   | "                      | "     | 32-47 <sup>(d)</sup>           |
| 7. Copper <sup>(g)</sup>   | "                      | "     | 68                             |
| 8. Gold                    | "                      | "     | 58-65 <sup>(d)</sup>           |
| 9. Iron <sup>(e)</sup>     | (h)Na salt             |       | 50-55                          |
|                            | 25 mole % acrylamide   |       |                                |
|                            | 75 mole % polyacrylate |       |                                |
| 10. Iron <sup>(h)</sup>    | "                      | "     | 42                             |
| 11. Copper <sup>(f)</sup>  | "                      | "     | 27-47 <sup>(d)</sup>           |
| 12. Copper <sup>(g)</sup>  | "                      | "     | 68                             |
| 13. Gold                   | "                      | "     | 70-75 <sup>(d)</sup>           |

<sup>(a)</sup>Eveleth

<sup>(b)</sup>Sherman

<sup>(c)</sup>Duval

<sup>(d)</sup>range of several samples

<sup>(e)</sup>Hanna

<sup>(f)</sup>Morenci

<sup>(g)</sup>Kingman

<sup>(h)</sup>polyacrylamide hydrolyzed to 75 mole % carboxylic acid

Substantial decreases in viscosity were also obtained with other concentrations and other polyacrylate-acrylamide copolymers in ratios of 1:1 and 1:3. Subsequent evaluations of those agents substantially reducing the viscosity of the ore slurries in ore grinding operations at the same or lower concentrations indicated surprising and significant increases in grinding kinetics.

#### EXAMPLE 2

A ball mill, 19.5 centimeters (cm) internal diameter and about 20 cm in length, operated at about 60 rpm and containing about 110 one-inch steel balls, was utilized for grinding studies on various ores to determine the effectiveness of using grinding aids of the present invention. In such operations, the ore was crushed and portions of the crushed ore passing through a 10 U.S. mesh screen were mixed with appropriate amounts of water in the mill to form slurries of desired concentrations. Once the desired slurry concentration was formed, the mill was sealed and operated for various grinding periods, after which the resultant ground ore slurry was removed and the amount of particles passing through a 325 U.S. mesh screen determined. The trials were then repeated, using the same concentrations and grinding times, with the addition of various amounts of a grinding aid to the aqueous slurry prior to grinding. The results of such operations, indicating the effectiveness of the grinding aid in improving grinding kinetics, are set forth below:

TABLE II

| Run No. | Grinding Aid | mg/gm Ore | Grinding Time mins | Wt. % Passing 325 Mesh | (a) % Increase | Ore Slurry %                               |
|---------|--------------|-----------|--------------------|------------------------|----------------|--------------------------------------------|
| 1.      | None         | 0         | 60                 | 47.0                   | —              | 84% taconite <sup>(b)</sup>                |
| 2.      | A            | 0.2       | 60                 | 51.5                   | 9.5            | "                                          |
| 3.      | A            | 0.4       | 60                 | 55.0                   | 17             | "                                          |
| 4.      | None         | 0         | 120                | 87.2                   | —              | 78% taconite <sup>(b)</sup>                |
| 5.      | A            | 0.15      | 120                | 89.5                   | 2.6            | "                                          |
| 6.      | None         | 0         | 40                 | 45.0                   | —              | 76% Copper <sup>(c)</sup>                  |
| 7.      | A            | 0.5       | 40                 | 47.0                   | 4.4            | "                                          |
| 8.      | A            | 2.0       | 40                 | 53.0                   | 13.3           | "                                          |
| 9.      | None         | 0         | 15                 | 25.5                   | —              | 78% Copper <sup>(d)</sup><br>(coarse feed) |

TABLE II-continued

| Run No. | Grinding Aid | mg/gm Ore | Grinding Time mins | Wt. % Passing 325 Mesh | (a) % Increase | Ore Slurry %              |
|---------|--------------|-----------|--------------------|------------------------|----------------|---------------------------|
| 10.     | A            | 0.2       | 15                 | 28.0                   | 9.8            | "                         |
| 11.     | None         | 0         | 30                 | 42.8                   | —              | 75% Copper <sup>(e)</sup> |
| 12.     | A            | 0.05      | 30                 | 44.1                   | 3.             | "                         |
| 13.     | A            | 0.15      | 30                 | 45.9                   | 7.2            | "                         |
| 14.     | A            | 0.5       | 30                 | 50.2                   | 17.3           | "                         |

A = sodium polyacrylate, molecular weight of from about 5000 to 10,000.

(a)

% increase as compared with control

(b) Mesabi Range ore

(c) Duval ore, feed = 9% <500 mesh

(d) Duval ore, coarse feed = 5% <500 mesh

(e) Morenci ore

The above data indicate that, with any fixed comparative grinding time, the weight percent passing 325 mesh is higher in all instances where a grinding aid was employed. A significant and surprising increase in the grinding kinetics was demonstrated even at low amounts of grinding aid (Run No. 5-2.6% increase with 0.015 weight percent of grinding aid), even where a relatively short grinding period was utilized (Run No. 12, 3% increase after 30 minutes with 0.005 weight percent grinding aid). Very dramatic and surprising increases in grinding are indicated for higher, but clearly economical, amounts of grinding aids. Increases of from about 10 to about 17% increases in the number and size of minus 325 mesh fragments being obtained with amounts ranging from 0.02 to 0.05 weight percent at grinding times of 15-60 minutes. Measurements at other particle sizes and ranges also indicated similar significant increases.

#### EXAMPLE 2

To further illustrate the effectiveness of the chemical grinding aids of the present invention on an industrial scale, reference is made to a trial conducted on taconite ore in an industrial scale overflow discharge rod grinding mill in which the ore was ground on a continuous circuit basis. In control grinding runs without the addition of a chemical grinding aid, an optimum range of grinding ore in an aqueous slurry without chemical addition to obtain a particle size less than 35 mesh (U.S. Standard) was obtained between 80 to 82% solids in the slurry. Any further increase in the percentage of solids in the slurry quite expectedly necessitated a reduction in the throughput of the ore ground in order to match the constant percent less than 35 mesh of the product. At an 86% solids density, the throughput falls off to about 400 tons per hour from a previous high of about 410 tons at a solids concentration of about 80 to 82%.

In grinding runs, a chemical grinding aid—sodium polyacrylate—was continuously added to the slurry in an amount of 0.13 lbs/ton of dry ore (0.065 mg/gm). The results were initially quite expected in that the addition of the grinding aid, at a concentration of 80 to 82% solids in the slurry, resulted in only a slight increase in throughput as compared to the control run in

which no grinding aid was added to the slurry. However, an unexpected and surprisingly sharp increase in the throughput was observed when the percent solids concentration of the slurry was raised to above 82%. At an 84% solids density, the throughput had increased to about 420 tons per hour while still maintaining the same percent less than 35 mesh in the product. At an 86% solids density, the throughput reached about 450 tons per hour, which represents an increase of about 10% over the 82% solids level of the control run.

An increase in the amount of the sodium polyacrylate grinding aid to about 0.20 lbs/ton was found to further increase the throughput, particularly at a percent solids concentration in the slurry of about 82-86%.

It is expected that a further increase in the percent solids concentration of the slurry above 86% will cause a gradual leveling off in the throughput and a subsequent fall-off at a percent solids concentration in the range above 90%. The actual trial was not conducted at a range above about 86% in order to avoid potentially serious problems in the operation of the rod mill caused by a tangling of the rods, a phenomena which is well known to persons skilled in the art.

Such data dramatically illustrate that the addition of the sodium polyacrylate grinding aid in this industrial scale trial in grinding taconite in a rod mill not only prevented a drop off in the throughput at a solids concentration above 82% but actually caused an increase in the throughput with an increase in the percent solids concentration of the slurry. This effect is completely unobvious and surprising in light of previous experience with grinding aids which were effective only to the extent of maintaining a relatively constant throughput with an increase in the percent solids concentration of the slurry, or which caused a slight increase in throughput but only with uneconomically large amounts of grinding aid chemical additions to the slurry.

#### EXAMPLE 3

In a laboratory scale batch test, taconite ore was ground in a mill in accordance with the procedure of Example 1. Sodium polyacrylate was evaluated as a grinding aid. The results are set forth in Table III.

TABLE III

| Runs <sup>(1)</sup> | Weight % Solids | Grams of Ore | Grams of Water | Sodium Polyacrylate (mg/gm) | # Grams Less than 325 mesh in Feed | # Grams Less than 325 mesh after 45 minutes |
|---------------------|-----------------|--------------|----------------|-----------------------------|------------------------------------|---------------------------------------------|
| 1                   | 80              | 1884         | 471            | —                           | 156                                | 1125                                        |
| 2                   | 82              | 1994         | 437            | —                           | 165                                | 1047                                        |
| 3                   | 84              | 2111         | 402            | —                           | 175                                | 969                                         |
| 4                   | 84              | 2111         | 402            | 0.19                        | 175                                | 990                                         |

TABLE III-continued

| Runs <sup>(1)</sup> | Weight % Solids | Grams of Ore | Grams of Water | Sodium Polyacrylate (mg/gm) | # Grams Less than 325 mesh in Feed | # Grams Less than 325 mesh after 45 minutes |
|---------------------|-----------------|--------------|----------------|-----------------------------|------------------------------------|---------------------------------------------|
| 5                   | 84              | 2111         | 402            | 0.28                        | 175                                | 1119                                        |

<sup>(1)</sup>All runs containing 0.5 mg of sodium silicate per gram of ore.

The foregoing data illustrates the effectiveness of the sodium polyacrylate grinding aid in Runs 4 and 5 in reversing the downward trend of fineness of grind of Runs 1 to 3 which were conducted without a grinding aid. As expected, with an increase in the weight percentage solids concentration in the aqueous slurry, the fineness of grind in the amount of ore ground decreases in Runs 1 to 3. However, the addition of the grinding aid at the relatively low concentration of only 0.19 mg/gm at the relatively high weight percent solids concentration resulted in an increase in fineness of grind. The further increase in fineness of grind was obtained in Run 5 with an increase in the amount of grinding aid to 0.28 mg/gm of ore.

#### EXAMPLE 4

In another laboratory scale batch test conducted in accordance with the procedure set forth in Example 1, sodium polyacrylate was evaluated as a grinding aid in the presence of a dispersant (sodium silicate) in the slurry. The results are set forth in Table IV.

TABLE IV

| Runs <sup>(1)</sup> | Weight % Solids | Grams of Ore | Grams of Water | Sodium Polyacrylate (mg/gm) | # Grams Less than 325 mesh in Feed | # Grams Less than 325 mesh after 30 minutes |
|---------------------|-----------------|--------------|----------------|-----------------------------|------------------------------------|---------------------------------------------|
| 1                   | 73              | 1500         | 448            | —                           | 278                                | 960                                         |
| 2                   | 75              | 1500         | 500            | —                           | 278                                | 870                                         |
| 3                   | 77              | 1500         | 554            | —                           | 278                                | 818                                         |
| 4                   | 77              | 1500         | 554            | 0.75                        | 278                                | 863                                         |

<sup>(1)</sup>All runs containing 0.5 mg of sodium silicate per gram of ore.

The table dramatically demonstrates that the use of sodium silicate as a dispersant in an amount of 0.5 mg/gm of copper ore in each of Runs 1 to 4 does not overcome the expected reduction in the fineness of grind of ore particles after grinding for 30 minutes that is experienced in purely aqueous systems. In each of Runs 1 to 3, it can be seen that with an increase in the percent solids (by weight) in the slurry, the fineness of grind declined from 960 grams to 818 grams of particles having a size less than 325 mesh. With the addition of the sodium polyacrylate grinding aid in Run 4, the decrease was reversed and a substantial improvement in fineness of grind was obtained at the high slurry solids content.

Other grinding aids of the invention are also similarly found to be effective in increasing the grinding kinetics with the above and other ore sources.

As will be apparent from the foregoing specification and examples, the best mode for carrying out the invention is as described in the preferred embodiments concerning the grinding aids, the amounts thereof, the grinding trials and result (grinding kinetic increases) determination procedures. The best mode known for carrying out the invention with a preferred grinding aid (sodium polyacrylate) on an industrial scale is as exemplified in Example 2 hereof. In additional efforts to optimize the use of the grinding aids of the present invention, preliminary trials indicate that the effective-

ness of a preferred grinding aid-sodium polyacrylate is enhanced if the pH of the slurry being ground is adjusted to higher levels, e.g., from about 8 to about 10 or more. Thus, in the grinding of certain ores where use of high slurry pH levels is beneficial and compatible with all aspects of the ore treating circuit concerned (i.e., flotation, etc.), such as the grinding of molybdenum, uranium, copper, etc., the best mode for using sodium polyacrylate appears to be in conjunction with the use of a base mixture of NaOH and Na<sub>2</sub>CO<sub>3</sub>.H<sub>2</sub>O. While synergistic grinding results from the use of a poly(meth)acrylic acid-sodium carbonate grinding aid system are separately disclosed in pending application Ser. No. 853,735, filed Nov. 21, 1977, and while use of the poly(meth)acrylic acid polymers with NaOH appears to result in increased grinding efficiency, the combined use of the grinding aid and two bases appears to give optimum results. Accordingly, where use of higher pH levels in a grinding circuit can be employed, it is believed the best presently known mode for using a grinding aid of the present invention is in conjunction with a

base mixture of NaOH and Na<sub>2</sub>CO<sub>3</sub>.H<sub>2</sub>O. Where sodium polyacrylate is the grinding aid and a taconite ore is being ground, it appears the best mode comprises the use of 0.2 mg of the grinding aid per gm of ore with from about 0.3 to about 0.4 mg of combined Na<sub>2</sub>CO<sub>3</sub>.H<sub>2</sub>O-NaOH base mixture (usually equal amounts of each) per gram of ore.

While this invention has been described with reference to certain specific embodiments, it is of course to be understood that the invention is not to be so limited except insofar as appear in the accompanying claims.

We claim:

1. A process for grinding coal or ores containing metal values comprising carrying out said grinding in the presence of a liquid medium and a polyelectrolyte grinding aid comprising acrylic or methacrylic acid polymers or copolymers of the same with each other or with other ethylenically unsaturated monomers, said grinding aid being dispersible in said medium and being employed in an amount effective to provide increased grinding efficiency.
2. The process of claim 1 wherein the grinding aid is a homopolymer of acrylic acid.
3. The process of claim 1 wherein the grinding aid is a homopolymer of methacrylic acid.
4. The process of claim 1 wherein the grinding aid comprises a copolymer of acrylic acid with an ethylenically unsaturated monomer.

5. The process of claim 1 wherein the grinding aid comprises a copolymer of methacrylic acid with an ethylenically unsaturated monomer.
6. The process of claim 1 wherein ores containing metal values are ground.
7. The process of claim 1 wherein coal is ground.
8. The process of claim 6 wherein the grinding aid is a homopolymer of acrylic acid.
9. The process of claim 6 wherein the grinding aid is a homopolymer of methacrylic acid.
10. The process of claim 7 wherein the grinding aid is a homopolymer of acrylic acid.
11. The process of claim 7 wherein the grinding aid is a homopolymer of methacrylic acid.
12. A process for grinding coal or ores containing metal values comprising carrying out said grinding in the presence of a liquid medium and a grinding aid comprising salts of acrylic or methacrylic acid polymers or copolymers of the same with each other or with other ethylenically unsaturated monomers, said grinding aid being dispersible in said medium and being employed in an amount effective to provide increased grinding efficiency.
13. The process of claim 12 wherein the grinding aid is a homopolymer of acrylic acid.

14. The process of claim 12 wherein the grinding aid is a homopolymer of methacrylic acid.
15. The process of claim 12 wherein the salt is an alkali metal or ammonium salt.
16. The process of claim 13 wherein the salt is an alkali metal or ammonium salt.
17. The process of claim 14 wherein the salt is an alkali metal or ammonium salt.
18. The process of claim 12 wherein the salt is an alkali metal.
19. The process of claim 18 wherein the alkali metal salt is sodium.
20. The process of claim 12 wherein the grinding aid is sodium polyacrylate.
21. The process of claim 12 wherein the grinding aid is sodium polymethacrylate.
22. The process of claim 12 wherein the grinding aid comprises a copolymer of acrylic acid with an ethylenically unsaturated monomer.
23. The process of claim 12 wherein the grinding aid comprises a copolymer of methacrylic acid with an ethylenically unsaturated monomer.
24. The process of claim 12 wherein coal is ground.
25. The process of claim 12 wherein ores containing metal values are ground.

\* \* \* \* \*

UNITED STATES PATENT AND TRADEMARK OFFICE  
CERTIFICATE OF CORRECTION

PATENT NO. : 4,162,044

DATED : July 24, 1979

INVENTOR(S) : Willy Manfroy and Richard R. Klimpel

It is certified that error appears in the above-identified patent and that said Letters Patent are hereby corrected as shown below:

Column 1, line 5, "Cross-Reference" misspelled;  
Column 3, lines 27 & 28, "methylacrylate" misspelled;  
Column 4, line 1, "polyelectrolyte" misspelled;  
Column 5, line 59, "chemical" should read "Chemical";  
Column 6, line 60, delete "50,00" and insert -- 50,000 -- ;  
Column 7, line 5 "determine" misspelled;  
Column 8, last line of Table I, delete "polyacrylamine"  
and insert -- polyacrylamide -- .

Signed and Sealed this

Thirteenth Day of November 1979

[SEAL]

Attest:

RUTH C. MASON  
*Attesting Officer*

LUTRELLE F. PARKER  
*Acting Commissioner of Patents and Trademarks*